

Jan. 21, 1941.

J. M. HOLM ET AL

2,229,208

GAS GENERATING CARTRIDGE

Filed Jan. 12, 1938



Fig. 3



Fig. 2



Fig. 1

John MacFie Holm  
William McEwen **INVENTORS**  
BY *Thos. A. Wilson*  
**ATTORNEY**

## UNITED STATES PATENT OFFICE

2,229,208

## GAS GENERATING CARTRIDGE

John Macfie Holm, Pollokshields, Glasgow, and  
William McEwen, Irvine, Ayrshire, Scotland,  
assignors to Imperial Chemical Industries Lim-  
ited, a corporation of Great Britain

Application January 12, 1938, Serial No. 184,700  
In Great Britain January 20, 1937

4 Claims. (Cl. 102—12)

The present invention relates to the provision of slow-burning gas-generating cartridges containing substantially ashless charges and suitable for use in conjunction with mechanical devices of the kind requiring for their operation the development of high pressures, e. g. of many hundred pounds per square inch, in a gradual manner. As examples of mechanical devices of this kind may be mentioned: high-pressure liquid-ejectors, engine starters, lorry-tipping devices, jacks, presses, electrical-switch-gear-operating devices, compressed-gas motors, brakes, and other devices operated by the motion of pistons.

The burning characteristics of ordinary propellant explosive compositions containing colloided nitrocellulose are such that attempts to employ cartridges of ordinary construction containing charges of this nature for the gradual generation of large pressures have hitherto failed to attain their objects. The rate at which the explosive burns in a confined space increases so rapidly as the pressure develops that the time occupied by the combustion of the whole charge seldom amounts to more than 2 seconds, and is usually a fraction of one second. Furthermore, the ratios of the maximum pressure to the final pressure developed increases so greatly with rise of loading density that in many cases such cartridges cannot produce large final pressures without imparting an undesirable shock to some part of the apparatus.

Our specification Serial No. 59,630 describes and claims composite charges and cartridges which are suitable for generating large pressures over a considerable number of seconds without developing unduly high ratios of maximum to final pressure. The charges or cartridges used according to the said specification include a charge element capable of self-propagating combustion when ignited at substantially atmospheric pressure, and one or more further charge elements capable of ignition only at pressures considerably in excess of atmospheric and generated by the combustion of the preceding charge elements, including the ignition means. In forming the charge elements, ordinary propellant explosive compositions are avoided; the use of these being confined to the initial part of the ignition train, which itself generates a pressure of not more than about 10 atm.

Pending application Serial No. 143,949 also describes a composite charge, for use in cartridges for similar purposes, in which at least one of the charge elements consisting of a compacted composition containing nitroguanidine.

Although the composite charges, and cartridges containing them, described in the two latter specifications are completely satisfactory for the purposes described, their production is inconvenient, in that the materials exemplified are hygroscopic or expensive.

This invention has as an object to provide a substantially ashless charge for cartridges of the type described which shall have none of the above mentioned disadvantages. A further object is to devise a method of manufacturing such charges. A further object is to provide a charge of this type which will be easy and economical to manufacture. Further objects will appear hereinafter.

These objects are accomplished by the following invention. We have now found that cartridges satisfactory for the purposes described, and capable of developing very considerable pressures at suitably slow rates without the development of unduly high ratios of maximum to final pressure, can be prepared advantageously from ordinary self-combustible ashless smokeless propellant explosive compositions, provided these are employed in solid rod form, and are protected from general superficial ignition by their flame gases by the method hereinafter described so that they burn only in the direction of their longitudinal axes.

According to the present invention, a slow-burning gas-generating cartridge or charge comprises a self-combustible substantially ashless propellant explosive composition in the form of a solid rod which is exposed to ignition at one end only, and is protected on its longitudinal surface by tightly wrapping around the rod in overlapping fashion a tape or sheet of material, forming in combination with an adhesion-promoting substance a closely adherent shield which prevents the contact of flame gases with the protected surface of the rod during the combustion thereof.

The propellant explosives used are preferably non-solvent propellants, e. g. solventless cordite or other double-base propellants. In some cases rods of propellants whose manufacture has involved the use of a volatile solvent may be employed; but, as the difficulty of producing homogeneous and sufficiently solvent-free rods of either single or double-base propellant of this type becomes extreme when the diameter of the rod finally produced exceeds about 1 cm.; and as the practical requirements in respect of gas volume and pressure required for successfully operating devices of the kind described, in conjunction with the characteristic burning speeds of solid propellant explosives, generally call for the use of rods

of greater diameter than 1 cm.; in practice a non-solvent propellant is to be preferred.

The wrapping material may conveniently consist of a fibrous or textile backing material, e.g. woven tape, paper, or the like, coated and/or impregnated with a cementitious adhesion-promoting material such as a cellulose derivative thermoplastic composition, a resinous composition, a rubber or rubber and oxidised oil composition, or a bituminous composition. The wrapping material may also consist of a homogeneous material such as cellulose acetate, regenerated cellulose, sheet rubber or the like; in which case the adhesion-promoting material may be a volatile solvent for the wrapping material and/or for the propellant itself.

Where the adhesion-promoting composition has a solvent effect on the rod, we prefer to apply a final coat of a varnish material that does not propagate its own combustion so that the shield does not lose its protective effect through impregnation with the propellant composition in solution:

In all cases the completed shield is such that  
25 it does not propagate its own combustion.

The means of ignition employed in association with the wrapped cylinder may consist of a percussion cap or an ordinary low-tension or high-tension fuzehead, in conjunction with priming means such as a small charge of propellant powder, or quick-match fuze or the like, in contact with the ignition end of the wrapped cylinder. In addition we may use a pellet or disc of a solid propellant composition as part of the priming means in order to ensure energetic ignition of the exposed end of the wrapped cylinder. This may be effected by leaving a short length unwrapped at the ignition end of the rod.

The cartridge case may be if desired constructed in relatively weak material such as paper, and the materials used in the manufacture of paper shotgun cartridge cases are suitable for use in carrying out our invention.

In use, the cartridges may be associated with a supporting metallic cage leaving a portion of the cartridge wall unsupported at some desired position, so that a vent for the combustion gases is formed by the rupture of the cartridge wall under the pressure produced by the combustion of the initiating means or of the initial portions of the charge. When initiated by a percussion cap of the usual kind, the cartridges may be arranged to vent near the base; and if initiated by electrical means, they may conveniently be arranged to vent at or near the forward end; in which case the use of a metallic supporting cage is unnecessary.

The use according to the present invention of wrapped cylinders of solid propellant explosive 60 as charges in gas-producing cartridges has the advantage that the burning speed does not vary irregularly and uncontrollably on account of destruction or displacement of the shield in the neighbourhood of the burning portion of the rod 65 so that flame gases penetrate through it or between it and the rod beyond the point of burning, and thus defeat the purpose for which the shield is employed.

Charges according to our invention may therefore be used without dependence on a tightly-fitting indestructible case as hitherto used; and if desired they may be used satisfactorily without any external protection other than that provided by the wrapping.

75 It will be understood that the distal end as well

as the cylindrical surface of the rod must be protected from premature ignition; and where the wrapped cylinder is used in conjunction with a cartridge case, a gas-tight fit of the wrapped cylinder in the case may be used to protect the distal end from leakage of flame gases between the wrapping and the case. We prefer, however, to apply a positive protection to the distal end surface so that a tight fit by the wrapped cartridge in the case is unnecessary. 10

In the attached drawing, Figures 1 and 2 are diagrammatic views in cross-section of cartridges venting near the base for use with percussion ignition. Figure 3 is a similar view of a cartridge arranged for forward ignition by means of an 15 electrical fuzehead. The invention is further illustrated in the following examples.

### Example 1

The charged cartridge of this example is illustrated in Figure 1. 20

An unlined paper cartridge case 1 having two 8 mm. diameter venting holes 16 mm. from the metal base 2 is employed. The external and internal diameters of the case correspond to 25 those of an ordinary 12 bore case, namely 19.9 mm. and 18.6 mm. respectively, but the length is somewhat greater. The ignition means are situated at the base of the cartridge and comprise the percussion cap 3, a priming charge 4 of 0.4 30 gm. Schultze gunpowder and 25 mm. quick-match 5 and a 1 gm. disc 6 of non-solvent Ardeer cordite 15.2 mm. in diameter having the composition: nitroglycerine 29%, nitrocellulose 65%, diethyl diphenyl urea 6%. The main charge 7 35 consists of 37 gm. of non-solvent Ardeer cordite rod of the same composition, 127 mm. long, 15.2 mm. in diameter, tightly wrapped from the ignition end with a 1700 mm. length 8 of adhesive electrical insulating tape 13 mm. wide and weighing 40 8.85 gm. per metre. A disc 9 of modelling clay is pressed on to one end of the rod and held in position by the projecting end of the tape. The wrapped rod is inserted into the cartridge case with the exposed end in contact with the Ardeer cordite disc, and the cartridge is closed 45 with a cardboard disc 10 and turnover 11.

When associated with a close-fitting cage having venting apertures registering with those of the cartridge case and tested by ignition in a closed vessel of 1050 c. c. capacity, the cartridge develops a maximum pressure of 780 lb. per sq. inch in about 40 seconds; the final pressure being 680 lb. per sq. inch.

*Example 2*

The cartridge of this example is illustrated in Figure 2.

An unlined paper cartridge case 1 having a metal base 2 provided with a 0.4 grain percussion cap 3 is employed. The external and internal diameters of the paper case correspond to those of an ordinary 12-bore case, namely 19.9 mm. and 18.6 mm. respectively, but the length is somewhat greater. The ignition means comprises the percussion cap, a priming charge 4 of 0.1 gm. Schultze gunpowder, a 150 mm. length of quick-match 5 and a 5.5 gm. pellet 6 of non-solvent Ardeer cordite 15.3 mm. in diameter and 20 mm. long; these being loaded at the base of the case. The composition of the Ardeer cordite is: nitroglycerine 38.5%; nitrocellulose 47.5%; moderants 14%. A white rubber disc 12 having an external diameter slightly greater than that of the case and 3 mm. thick is placed between the igniting 75

means and the main charge 1, this disc having a central perforation 7 mm. in diameter. The main charge consists of a rod 120 mm. in length of the same Ardeer cordite composition weighing 33.5 gm., wrapped in overlapping spiral fashion, starting from the ignition end, with a 1100 mm. length 8 of adhesive electrical insulating tape 13 mm. wide and weighing 8.85 gm. per metre. The remote end of the charge from the igniting means 10 is protected by a prolongation of the spiral wrapping folded over and pressed against the end surface. The wrapped rod is inserted into the cartridge case with the exposed end in contact with the white rubber disc, which protects the wrapped 15 longitudinal surface from the combustion gases generated by the igniting means, while leaving the end surface in ignition contact therewith through the central hole. The case is closed by a  $\frac{1}{8}$  inch cardboard disc 10, secured by the usual 20 type of shotgun cartridge case turnover 11. When tested in the manner described in Example 1 in a closed vessel of 570 cc. capacity the cartridge develops a maximum pressure of about 1800 lb./sq. in. in a gradual manner in 25 seconds, 25 the final pressure being about 1500 lb./sq. in.

*Example 3*

In this example the cartridge case, ignition means and white rubber disc are as described 30 above in Example 2. The main charge consists of a 130 mm. length of the same Ardeer cordite as used in Example 2 weighing 36.2 gm. and wrapped with two spiral layers of surgical adhesive tape, the length employed being 2000 mm. 35 and the width 12.5 mm. This tape weighs 2.1 gm. per metre. One end of the charge is protected by folding over a prolongation of the spiral wrapping and pressing it against the end surface. The charge is loaded in the case and the case closed as described above in Example 2. 40 When tested in the manner described in Example 1 in a closed vessel of 1050 c. c. capacity, a maximum pressure of about 1000 lb./sq. in. is developed by the cartridge in 36 seconds; the final pressure being about 900 lb./sq. in. 45

*Example 4*

The cartridge case, cap, and white rubber disc in this example are as described in Example 2. In addition to the percussion cap, the priming 50 means includes 0.4 gm. of Schultze gunpowder, a 150 mm. length of quickmatch, and a 12.5 mm. length of Ardeer cordite 15.2 mm. in diameter and weighing 3.7 gm. This Ardeer cordite 55 has the composition, nitroglycerine 30%; nitrocellulose 64%; and diethyl diphenyl urea 6%. The main charge consists of 127 mm. of this same Ardeer cordite wrapped round in spiral fashion with a 500 mm. length of grey adhesive rubber tape, 19.3 mm. wide, 0.8 mm. thick and weighing 60 27.7 gm. per metre. One end of the charge is protected by folding over a prolongation of the spiral wrapping and pressing it against the end surface. This charge is loaded and the case closed as described in the previous examples. 65 When tested in the manner described in Example 1 in a closed vessel of 1050 cc. capacity a maximum pressure of about 860 lb./sq. inch is developed in 33 seconds, the final pressure being 700 lbs./sq. in. 70

*Example 5*

In this example the cartridge case, ignition means and white rubber disc are the same as employed in Example 2. The main charge consists 75 of 76 mm. of the same Ardeer cordite as em-

ployed in Example 2 and weighs 21.2 gm. It is wrapped in a spiral fashion with 620 mm. of a masking paper tape 25 mm. wide and weighing 4.9 gm. per metre having a coating of a thermoplastic adhesive. One end of the main charge is 5 protected by folding over a prolongation of the spiral wrapping and pressing it against the end surface. This charge is loaded and the case closed as described in Example 2. When tested as in Example 1 in a closed vessel of 1260 cc. 10 capacity the cartridge develops a maximum pressure of about 420 lb./sq. in. in 33 seconds, the final pressure being about 400 lb./sq. in.

*Example 6*

15

The cartridge case is as in Example 2 and the ignition from the percussion cap is transmitted through 0.45 gm. Schultze gunpowder and a 250 mm. length of quickmatch to a 4 gm. disc of an Ardeer cordite having the composition nitro-glycerine 29%; nitrocellulose 65%; diethyl diphenyl urea 6%. The main charge consists of a protected rod of Ardeer cordite of a different composition, namely that used according to Example 2, the rod being 15.3 mm. in diameter, 25 76 mm. long and weighing 21 gm. in its unwrapped state. The rod is protected by dipping it in acetone and winding it tightly with a strip of acetone-soluble cellulose acetate 96 mm. broad and 0.22 mm. thick and somewhat longer than 30 the rod, the overlap being sealed with the aid of acetone.

One end of the wrapped rod is sealed off with modelling clay and the rod is inserted with the exposed end in contact with the 4 gm. disc. 35 When tested in the manner described in Example 1 the cartridge produces a maximum pressure of 425 lb./sq. in. in 32½ secs., the final pressure being 400 lb./sq. in.

*Example 7*

40

This example describes the cartridge adapted for forward ignition and illustrated in Figure 3.

The charge consists of a solid homogeneous cylinder 7 of solventless cordite 108 mm. long, 23 mm. diameter and weighing 67 gm., and consisting of nitroglycerine 35.5%, nitrocellulose 51%, diethyl-diphenylurea 5%, diethyl phthalate 7% and potassium nitrate 1.5%. A 1400 mm. length of tape 8 which is 13 mm. wide and is impregnated with an adhesive castor-oil rubber composition, is wound tightly round the rod in an overlapping spiral so that 10 mm. at one end of the rod is left uncovered; the other end being sealed off by a disc of similar adhesive tape over which the projection portion of the wrapping is turned down. The wrapped cylinder is inserted, sealed end foremost, into a paper shotgun cartridge case 1 which is 26 mm. in external diameter, 24.5 mm. internal diameter, and 130 mm. long. The case is fitted with a brass shell 2 having an insulated central electrode 14. The means of ignition consists of an ordinary low-tension electric fuzehead 17, whose insulated leads 13 are connected to the brass base and the central electrode respectively and are led forward between the case and the wrapped cylinder so that the fuzehead is in contact with the exposed end of the rod. A 33 mm. length of quickmatch fuze 5 weighing 0.22 gm. and 0.1 gm. of Schultze gunpowder 4 are also loaded in contact with the exposed end of the rod, and the case is closed by a Celluloid disc 10, which is 24.5 mm. in diameter and 0.5 mm. thick, and the usual type of shotgun case turnover 11. 70

75

When the cartridge is loaded directly in the breech of a closed test vessel of about 1330 ml. capacity and the fuzehead fired by the application of a suitable firing current, a maximum pressure of about 1300 lb./sq. inch is gradually developed in about 25 seconds; the final pressure being about 870 lb./sq. inch.

*Example 8*

10 This example illustrates the use of an unenclosed wrapped charge.

A 280 mm. by 7 mm. diameter rod of solventless cordite weighing 19.3 gm. and consisting of nitro-glycerine 41%, nitrocellulose 52% and diethylidiphenylurea 7% is wrapped in a double overlapping spiral of 730 mm. of a textile adhesive tape as described in Example 4. 25 mm. of the rod is left exposed at one end, and the other end is protected by folding over the projecting portion of the adhesive tape 50 mm. of quickmatch tape 6 mm. wide and a low-tension electric fuzehead are bound to the exposed end of the rod with cotton thread, and the insulated fuzehead leads are connected to the firing terminals of a closed testing vessel of 1 litre capacity.

When fired inside the vessel, the charge produces a very gradual rise of pressure to a maximum of 800 lb./sq. in. in about 72 seconds; the final pressure being about 750 lb./sq. inch.

30 As many apparently widely different embodiments of this invention may be made without de-

parting from the spirit and scope thereof, it is to be understood that we do not limit ourselves to the specific embodiments thereof, except as defined in the appended claims.

We claim:

1. A slow burning gas generating cartridge comprising a solid rod of a self-combustible, substantially ashless propellant explosive composition, and a non-metallic shield covering the longitudinal surface of said rod, said shield being of such composition as to prevent the contact of flame gases with said covered surface during combustion and comprising a layer of non-metallic imperforate sheet material in combination with an adhesion promoting substance disposed in close contact with said rod, and ignition means associated with said cartridge, one end only of said rod being exposed thereto.

2. The cartridge of claim 1 wherein the shield comprises a non-metallic fibrous backing material in combination with an adhesion promoting substance.

3. The cartridge of claim 1 wherein the shield comprises regenerated cellulose in combination with an adhesion promoting material.

4. The cartridge of claim 1 wherein the shield comprises cellulose acetate in combination with an adhesion promoting material.

JOHN MACFIE HOLM. 30  
WILLIAM McEWEN.